

## UNITED STATES PATENT OFFICE

2,081,075

## LUBRICATING OIL COMPOSITION

Arnold C. Vobach, Whiting, Ind., assignor to  
Sinclair Refining Company, New York, N. Y.,  
a corporation of Maine

No Drawing. Application July 6, 1936,  
Serial No. 89,120

6 Claims. (Cl. 87-9)

My invention relates to improvements in compounded petroleum lubricating oils. The improved lubricating oil compositions of my invention consist essentially of a petroleum lubricating oil and calcium phenyl stearate, or calcium phenyl stearate together with calcium stearate, or calcium phenyl stearate or a mixture of calcium phenyl stearate and calcium stearate together with phenyl stearic acid, in amount, or amounts, insufficient materially to alter the normally liquid character of the petroleum lubricating oil itself, 0.5-2.5% on the oil for example.

Calcium phenyl stearate, and its production, have been described in the chemical literature, see for example Journal of the American Chemical Society, 49, 1103-1106, (1927), and 52, 1172-1174, (1930). Calcium stearate has long been used in compounded petroleum lubricating greases. This invention relates to improvements in liquid petroleum lubricants as distinguished from solid or semi-solid petroleum greases. The term "petroleum lubricating oils" is intended to refer herein to lubricating oils of petroleum origin having viscosities upwards of 50-70 seconds at 100° F. Saybolt universal.

The trend of development in internal combustion engines has imposed increasing burdens upon the oils used for their lubrication, particularly with respect to operating temperatures and pressures. At present, the Diesel type of engine probably represents extreme requirements in both of these respects, but it is not alone in the imposition of severe burdens upon the lubricating oil used. The useful operating life of a lubricating oil, in such service, is determined, in large measure, by its thermal stability and by its physical capacity to continue functioning as a lubricant, at the high temperatures and high pressures encountered. One measure of thermal stability is resistance to oxidation, and the consequent tendency to form sludge, but in another aspect the effect of thermal instability is determined not only by the extent of oxidation or decomposition but also by the character of the products of such decomposition or oxidation and by the extent and location, within the engine, of deposits of such products.

The improved lubricating oil compositions of my invention have, in addition to the lubricating properties of the petroleum oils of which they are

compounded, a high solvent capacity for sludge, of the character formed by oxidation of petroleum lubricating oils and, perhaps of even greater importance, the properties of rendering deposits of sludge and "carbon" within the engine soft and friable rather than hard and coherent and of disintegrating and removing such deposits as an incident of the normal operation of the engine. In this aspect, the lubricating oil compositions of my invention render the engines in which they are used self-cleaning to an important extent.

In the Diesel type of engine, for example, the high temperatures to which the lubricating oil is subjected, particularly at the top of the stroke, frequently causes deposition of sludge and carbonization in the groove for and behind one or more of the piston rings. Using paraffinic type lubricating oils such difficulties are usually more pronounced with respect to the uppermost ring; using naphthenic type lubricating oil they are usually more pronounced with respect to the lower rings. Consequent sticking of the rings rapidly deprives the piston and cylinder wall of proper lubrication inducing excessive wear and, frequently, scoring of the cylinder wall. The formation of such "carbon" deposits, hard enough and coherent enough to involve sticking of the rings, is materially retarded, if not avoided, by the use of the improved lubricating oil compositions of my invention, and in this aspect the self-cleaning properties of the lubricating oil compositions of my invention, with respect to the engine, make a mere change of oil a substitute, economical with respect both to loss of service time and cost, for many otherwise necessary cleaning and repair jobs.

Calcium phenyl stearate, or mixtures including calcium phenyl stearate and calcium stearate, for compounding the improved lubricating oil compositions of my invention can be produced as follows: 1 part (parts by weight) of pulverulent anhydrous aluminum chloride is stirred into 4 parts of commercial benzol boiling 90% below 100° C., this stirring being effected at atmospheric pressure and at ordinary temperature. 2 parts of oleic acid, commercial red oil containing as a minimum 96% free fatty acid as oleic acid and having a maximum cloud test of 45° F., is added to this mixture with stirring, the addition being made over a period of about an hour. This re-

action is carried out at atmospheric pressure and is started at ordinary temperature. The temperature rise incident to the reaction is limited so that the maximum temperature approximates 5 180° F., the temperature being controlled either by cooling or by regulating the rate of addition of the oleic acid. The reaction mixture is maintained at a temperature of 140°-180° F. for 6 or 7 hours. For at least the last half hour of this 10 period the reaction mixture is held at 180° F. to insure completion of the reaction and to assist in stripping hydrochloric acid from the reaction mixture. The reaction product, a pasty liquid, is then added to about  $\frac{1}{4}$  of its volume of aqueous hydrochloric acid, 20% HCl, at ordinary temperature. The ensuing reaction brings the temperature, for example, to about 170° F. This reaction mixture is thoroughly stirred and the aqueous acid solution is then separated from the 15 oily product of the reaction, by decantation for example. This separated oily product is thoroughly washed with water, advantageously with hot water, in two successive stages with about  $\frac{1}{2}$  of its volume of hot water in each stage for 20 example. This washing should in any event be continued until a quantitative test for aluminum in the wash water is negative. After this washing, the reaction product is a thin, oily, dark green liquid. It is allowed to stand to settle out 25 any remaining water. Benzol is stripped from this oily liquid by distillation, limiting the maximum liquid temperature to about 350° F., using steam or other distillation medium to effect the stripping within this maximum temperature limit. The oily liquid remaining after stripping of benzol is then subjected to distillation, advantageously under a high vacuum, 2-4 millimeters of mercury absolute pressure for example. This distillation may be otherwise effected, using 30 steam or other distillation medium for example, provided the material undergoing distillation is not heated to any temperature much exceeding 640°-650° F. for any period long enough to involve decomposition. When effecting the distillation under a vacuum of 4 millimeters of mercury absolute pressure, a first cut of about 25% is taken off up to the point at which the temperature of the liquid in the still reaches 466° F. and a second cut of about 53% is taken off as the 35 temperature of the liquid in the still rises from 466° F. to 590° F. The second of these two distillate fractions can be saponified with lime to produce the material to which I refer as calcium phenyl stearate, or these two distillate fractions 40 can be combined and together saponified with lime to produce a mixture of this calcium phenyl stearate and calcium stearate. For example, 4 parts of the second fraction, or 4 parts of the first and second fractions together, diluted with an equal weight of petroleum naphtha boiling between about 200° F. and 322° F., can be saponified with about 1 part of hydrated lime, added in 2 or 45 3 portions with thorough stirring. The temperature of the reaction mixture rises to about 160° F., for example, and then by external heating with reflux condensation of the naphtha diluent is maintained at about 190° F. until the saponification is complete. This reaction mixture is further diluted with about twice its volume of the 50 same petroleum naphtha and unreacted lime is separated by centrifuging. Benzol may be used, as a diluent, in both instances, in place of naphtha. After separation of unreacted lime, the diluent is distilled off, limiting the maximum temperature of the liquid in the still to about 375° F., 55

carrying out the distillation under a vacuum if necessary to keep within this temperature limitation. This undistilled liquid product is used as calcium phenyl stearate, or as a mixture of calcium phenyl stearate and calcium stearate if 5 the first distillate fraction as well as the second is saponified, in compounding the improved lubricating oil compositions of my invention. Instead of saponifying the second distillate fraction, or the first and second distillate fractions 10 as just described, a somewhat larger excess of lime may be used, 3 parts of the distillate fraction or fractions to 1 part of hydrated lime for example without dilution until the saponification is completed and the reaction mixture then diluted prior to separation of unreacted lime, the saponification being otherwise carried out as just described. Or, it is also possible to use that amount of hydrated lime just necessary to complete the saponification, and to effect the saponification without dilution either during the saponification or following the saponification. 15 20

In referring to "phenyl stearic acid" herein, I refer to the calcium compound constituting the major component of the saponification of the second distillate fraction from the condensation of oleic acid with benzol as described in the preceding paragraph although, of course, I intend to refer by this term to this same material by whatever process it may be made. I believe this 25 calcium phenyl stearate to be the calcium salt of 9,10 phenyl stearic acid, but I do not predicate my invention upon this identification of the compound as a matter of terminology. The refractive indices, acid numbers, saponification numbers and iodine numbers of the total reaction 30 product of the oleic acid-benzol condensation, of the first and second distillate fractions and of the residual fraction produced as described in the preceding paragraph, as determined in one instance, were as follows: 35 40

|                            | Total reaction product | First cut | Second cut | Residue | 45 |
|----------------------------|------------------------|-----------|------------|---------|----|
| Refractive index at 20° C. | 1.4875                 | 1.4610    | 1.4880     | 1.5171  |    |
| Acid number                | 166                    | 193       | 155        | 127.5   |    |
| Saponification number      | 168.1                  | 192.6     | 160        | 161.7   |    |
| Iodine number              | 10                     | 1.96      | 4.08       | 23.6    | 50 |

In compounding the improved lubricating oil compositions of my invention with the usual petroleum lubricating oils, the calcium phenyl stearate, or the mixture including calcium phenyl stearate and calcium stearate, are added to the lubricating oil in proportions ranging from about 0.5% up to about 2.0% or 2.5% by weight on the oil. I have found a composition consisting essentially of a South Texas pale oil, having a viscosity of 500 seconds at 100° F., Saybolt universal and 55 boiling 10% up to 700° F. and 90% up to 900° F., approximately, and 1  $\frac{1}{3}$  % by weight on the oil of a mixture of calcium phenyl stearate and calcium stearate produced by saponifying together the first and second distillate fractions from the vacuum distillation of the reaction mixture from the condensation of oleic acid with benzol as described in the second preceding paragraph to be particularly advantageous. The "Indiana Oxidation Test" with this composition was 24-25 hours 60 as compared to 14 hours for the petroleum lubricating oil alone. This Indiana Oxidation Test is described in the S. A. E. Journal, 34, 172-173 (1934). In service in a Diesel type engine, this lubricating oil composition left the engine free 65 70 75

from sludge or carbon deposits except for a slight discoloration of the piston just above the lowermost compression ring and adequately lubricated the moving parts of the engine. The properties 5 of this particular lubricating oil composition, as compared to that of the petroleum lubricating oil alone, as determined in one instance, were as follows:

|    |                                              |                 |                                                                        |
|----|----------------------------------------------|-----------------|------------------------------------------------------------------------|
| 10 |                                              | South Texas oil | South Texas oil + 13 1/2% calcium phenyl stearate and calcium stearate |
| 15 | Gravity.....                                 | 20.7 A. P. I.   | 20.8 A. P. I.                                                          |
|    | Flash.....                                   | 375° F.         | 370° F.                                                                |
|    | Fire.....                                    | 420° F.         | 415° F.                                                                |
|    | Viscosity at 100° F., Saybolt universal..... | 506 seconds.    | 525 seconds.                                                           |
| 20 | Viscosity at 210° F., Saybolt universal..... | 53.5 seconds.   | 54.8 seconds.                                                          |
|    | Pour.....                                    | -10° F.         | -15° F.                                                                |
|    | Carbon Residue.....                          | 0.041.          | 0.088.                                                                 |
|    | Ash.....                                     | 0.001.          | 0.115.                                                                 |
|    | Acid Number.....                             | 0.059.          | 0.475.                                                                 |
|    | Saponification Number.....                   | 0.423.          | 2.54.                                                                  |

25 While the lubricating oil composition of the foregoing example embodies specifically a South Texas lubricating oil, my invention is also useful in lubricating oil compositions embodying petroleum lubricating oil from paraffin base crudes, asphaltic base crudes and mixed base crudes.

For some purposes, the properties of the compounded lubricating oil of my invention may be improved by stopping the saponification of the phenyl stearic acid, or phenyl stearic acid mixture, somewhat short of completion to produce a calcium phenyl stearate mixture including a minor proportion, 7% of the total mixture for example, of phenyl stearic acid and adding this mixture including some unsaponified phenyl stearic acid to the petroleum lubricating oil in proportions ranging from about 0.5% up to about 2.5% by weight on the oil. The presence of unsaponified phenyl stearic acid in the mixture reduces any tendency of the compounding agent 45 abnormally to increase the viscosity of the oil to which it is added, and may with some oils improve the viscosity index. The foregoing proportion of free phenyl stearic acid in the mixture is particularly advantageous; it may be usefully included in proportions up to about 20% of the total mixture. Instead of stopping the saponification short of completion, free phenyl stearic acid may be added to calcium phenyl stearate to produce similar mixtures.

55 While I predicate my invention upon the re-

sults obtained in its practical application, and not upon any hypothesis, it now appears that the calcium soaps of aromatic stearic acids, generally, are useful for the purposes of my invention. Other aromatic stearic acids, tolyl stearic acid, xylyl stearic acid, naphthyl stearic acid, and anthracyl stearic acid for example, may be made by methods generally similar to the method above described for the production of phenyl stearic acid, and may similarly be saponified with lime 10 to produce the corresponding calcium soaps. The presence of the aromatic group in the calcium soap seems to promote the solvent capacity of the lubricating oil composition with respect to sludge, and may assist in improving its thermal 15 stability. Soaps of these organic acids containing an aromatic group also have the property of decomposing at a temperature approximating the end point, or carbonization temperature, of the petroleum lubricating oils used in the lubricating 20 oil compositions of my invention. I do not at present know with certainty what if any relation may exist between this property and the properties of the improved lubricating oils of my invention of rendering deposits of carbon and sludge 25 within the engine soft and friable and disintegrating such deposits, but I believe them to be closely related to each other and to the bringing of the calcium oxide equivalent of the calcium soap into the regions within the engine in which such deposits occur and might otherwise remain 30 in a form effective to give the lubricating oil composition of my invention these properties.

I claim:

1. A liquid lubricating oil composition comprising a petroleum lubricating oil and calcium phenyl stearate.
2. A liquid lubricating oil composition comprising a petroleum lubricating oil, calcium phenyl stearate and calcium stearate.
3. A liquid lubricating oil composition comprising a petroleum lubricating oil, calcium phenyl stearate and phenyl stearic acid.
4. A liquid lubricating oil composition comprising a petroleum lubricating oil, calcium phenyl stearate, calcium stearate and phenyl stearic acid.
5. A liquid lubricating oil composition comprising a petroleum lubricating oil and a calcium soap of a stearic acid containing an aromatic group, said soap having a decomposition temperature approximating the end point of said oil.
6. A liquid lubricating oil composition comprising a petroleum lubricating oil and a calcium soap of an aromatic stearic acid.

ARNOLD C. VOBACH. 55